

June 29, 1926.

1,590,593

E. TAYLOR ET AL

## CONVERSION OF CELLULAR OR FIBROUS MATERIAL

Filed Dec. 2, 1919



## UNITED STATES PATENT OFFICE.

EDWIN TAYLOR AND EDWARD F. CHANDLER, OF BROOKLYN, NEW YORK, ASSIGNEES,  
BY MESNE ASSIGNMENTS, TO TAYLOR LABORATORIES INC., OF NEW YORK, N. Y., A  
CORPORATION OF NEW YORK.

## CONVERSION OF CELLULAR OR FIBROUS MATERIAL.

Application filed December 2, 1919. Serial No. 341,953.

The invention relates to improvements in the conversion of cellulose or fibrous material. In our prior co-pending application for United States Letters Patent, Serial No. 5 314,102, filed July 29, 1919, we have described a process wherein organic material such as cellulose in a fibrous or cellular condition may be converted by dissolving the cellulose in a suitable solvent, such as cupro-10 ammonia solution and electrolyzing the solution between a suitable anode and cathode whereby cellulose substantially free of the solvent chemicals is deposited on the anode and the copper is deposited on the 15 cathode and ammonia is freed. The main object of the present invention is to provide improvements whereby such organic matter may be so treated more expeditiously and in a more economical and useful manner. 20 Further and more specific objects, features and advantages will more clearly appear from the detail description given below.

In the preferred method of practicing the inventive idea the organic or cellulose material to be converted is dissolved preferably in an excess of cupro-ammonia solution, filtered to remove extraneous impurities, the solution concentrated by the partial removal of ammonia and water (as for instance by 30 means of a vacuum), the resulting homogeneous fluid flowed on a carrier which may be a flexible band of metal suitable for employment as one of the elements of an electrolytic cell, the said carrier being adapted to convey the flowed material through preferably a dry and inert gas, thereby excluding deleterious atmospheric contamination. The carrier conveying the flowed material now enters and becomes preferably one of 40 the elements or electrodes, in a bath which may be provided with another element or electrode so as to constitute an electrolytic cell upon the energization of the said elements and through which the carrier which 45 may be the anode, is adapted to continuously convey the flowed material. Owing to the electrolytic characteristics of cellulose in a colloidal state, the flowed material as it passes through the influence of the said electric field or fields is converted from the colloidal solution to a solid or more dense 50 state which transformation should be com-

pleted under proper conditions of time and current density before the carrier and material leaves the cell. During the period of 55 transformation the volatile constituent is released from the mass and is in a condition to be conveyed to a suitable condensing or recovering system, the metallic constituent being deposited on the cathode in recoverable condition. The transformed organic material free of all traces of any ingredient that might cause future deterioration is preferably conveyed through a suitable washing system where any adhering or extraneous traces of foreign materials are removed and thence to a suitable drying system for the removal of any moisture content after which the converted material is ready 65 for separation from the conveyer or carrier. This separation may be effected by means of a V-shaped fixed edge supplemented by two rolls.

The material, now in a transparent flexible band resembling celluloid in appearance 75 is then led through a bath containing a volatile solvent such as amyl-acetate which possesses a slight solvent or softening effect on the cellulose and materially aids in increasing its surface lustre, its density, and its resistance to moisture. The material still wet with solvent is now passed through warm calender rolls whereon it is surfaced, brought to exact thickness and dried and the solvent recovered. From the calenders 80 the finished product may be wound on reels, cut or trimmed in sheets or strips or otherwise disposed of.

It will be seen that this process is economical, as well as continuous. All the solvent materials are recovered in usable form 90 for re-solution, even the trimmings from the finished material being returned to the solution tanks. The power factor is low and the amount of labor required is almost negligible. It is evident that the above process can be advantageously carried out 95 by the use of a concentrated zinc chloride solution, etc., in place of the cupro-ammonia.

In the accompanying drawings we have 100 illustrated a suitable application of our invention as applied to the manufacturing of photographic films. In said drawings, Fig.

1 illustrates in vertical cross-section, parts being broken away, the arrangement of a suitable plant for manufacturing photographic films, and Fig. 2 is an enlarged 5 cross-sectional detail of the endless belt and film formed thereon.

3-4 indicate suitable tanks carrying concentrated solution of cupro-ammonia or concentrated solution of zinc chloride both 10 being good solvents for cotton which may be used in the manufacturing of the film. About one pound of cotton may be used to about twenty pounds of the solution and suitable means such as the valve 5 may be 15 provided for regulating the flow of the material upon the endless belt 6 which passes entirely through the closed tray or chamber 7 as shown.

The belt may be made of copper and may 20 be plated with other metal and buffed and may be suitably perforated as indicated at 8 in Fig. 2 to receive the teeth of sprocket wheels for driving the same, suitable means for driving the belt being provided such as 25 9, an electric motor connected to the driving shaft 10. Upon the belt may be provided suitable strips of material such as 11 between which the flowing material from the tanks 3-4 is deposited. In the drawing 30 I have illustrated the belt as traveling from left to right looking at Fig. 1.

The ammonia from the closed tray 7 is 35 drawn through the outlet pipe 12 by the suction fan 13 and is passed through the drying chamber 14 provided with suitable grids 15 upon which lime or other suitable material 15' may be piled, the dry ammonia returning through the pipe 16 into the closed tray 7 as shown. This provides a constant 40 circulation of dry ammonia gas in the closed chamber 7 and prevents waste of material and contamination from the outside.

17 indicates an electrolytic cell to be hereafter more fully referred to and is in communication with the superimposed chamber 18 through which ammonia, hydrogen, oxygen or other gases rise and escape by way of the pipe 19 controlled by the valve 20 into the chamber 21 escaping under the hood 22 50 for condensation and recovery except when the valve 23 is open to allow the same to pass to the drying chamber 14.

The electrolytic bath 17 may be provided with copper electrodes 24 or when the process 55 is worked with zinc chloride, zinc electrodes may be used. An acidulated solution of nitric or sulphuric acid 25 is provided as an electrolyte sufficiently strong to carry the current.

60 As the cellulose fed upon the belt 6 passes down through the chamber 18, it passes beneath the first electrode 24 at the right side of the figure over the pulley 26, beneath the next electrode, over the next pulley and so 55 on until it enters the chamber 27, said pul-

leys being driven by the worms 28 upon the motor shaft 10 and said electrodes being connected to the negative side of a suitable source of electricity as shown, with the result that the metallic content of the cellulose upon the belt is electrodeposited therefrom 70

upon the electrodes 24 leaving the cellulose gradually becoming white instead of blue or green as it passes through the electrolytic bath until upon leaving said bath the cellulose is quite white, whereupon it enters the washing tank 27 before referred to. The film is now sufficiently tough and flexible for washing whereas if the metallic content remained in the film, it would upon drying be 80

brittle and liable to break up. In the washing tank 27 water enters by the pipe 29 controlled by the valve 30 and escapes by the pipe 31 which may be provided with a valve 32, the film passing over the pulleys 33

driven by the worms 34 upon the said motor shaft 10, and a suitable partition 35 may be provided with an opening at the bottom as indicated at 36 so as bring the film in contact with the cleaner water of the wash as 90

it leaves the tank 27. All of these tanks are preferably closed to prevent foreign matter from coming in contact with the film and if desired suitable means may be provided for 95 evacuating air therefrom as any carbonic acid present in the room is apt to form carbonate, this especially applies to the drying tank and various other objectionable results may be encountered. The washing tank removes any adhering ammonia, acid, 100

of particles of matter, after which the film passes to the drying chamber 37 where it again passes over pulleys such as 38 driven by worms such as 39 and beneath pulleys such as 40 until it finally emerges over the 105 pulley 41 as shown. This drying tank may of course be heated by any suitable means to a temperature, say perhaps 120 degrees Fahrenheit. The film is now loosened from the belt upon which it was formed and due 110

to the heat, shrinkage, etc., is readily separated therefrom, and in this connection a suitable knife or stripper such as 42 may be provided adjacent the periphery of the roll 41 so as to allow the film to pass leftwardly 115 between the rollers 43 of the tank 44 while the belt or carrier passes downwardly beneath the pulleys 45 from which point it returns to the starting place and again passes through the closed tray 7.

The detached film upon entering the tank 44 passes over the roller 46 driven by the worm 47 and downwardly through the amyl acetate bath 48 passing upwardly again over the roller 49 and upon the rolls 50 preferably 125 of highly polished surface. In the amyl acetate tank the film is softened, densified, and is increased in its resistance to moisture, after which, upon passing first leftwardly around the top roll 50, then rightwardly 130

around the next roll below, and leftwardly again, and so on alternately, it becomes thoroughly dried and finished and is wound upon the reel 51, while the amyacetate vapors escaping through the outlet 52 may be condensed for re-use, thus providing a continuous, economic, and practical method of producing film in which there are practically no losses, but complete recovery of materials, the film being adapted to travel through the system with a speed of production higher than in any of the present well known methods, while at the same time producing a film of greater transparency and durability, one which is practically non-combustible and of numerous other properties and advantages.

One of the advantages in the use of our film for photographic purposes is that it may be impregnated from one side (preferably uncalendered) with a solution of silver salt, such as nitrate of silver, after which the film may be exposed to an atmosphere of, and impregnated with bromine, chlorine, iodine or a combination thereof, thereby depositing insoluble bromide or chloride etc. of silver in the film itself. It will be found that by preparing photographic films in this manner that after the same has been photographically exposed and developed there is no flaking off or scratching off of the negative surface, thus preventing the objectionable effects in photography so much complained of, as even if the surface of our film be scratched or mutilated, the chemicals having penetrated the film, still present the photographic image, which in the path of the light registers the characters, notwithstanding the mutilated surface of the film.

Another advantage of our process resides in the fact that by passing the film from the drying chamber 37 through any well known form of nitrate bath of any desired consistency, a pyroxylene may be obtained in a dense continuous sheet having the same nitrogen content as the original cotton immersed under equal conditions in the same bath. This provides a ready means for manufacturing granulated smokeless powder without the use of a volatile solvent.

The cupro-ammonia solution hereinbefore referred to is preferably made by dissolving hydrated cupric-oxide  $CuH_2O_2$  in approximately an equal weight of ammonia water containing thirty per cent (30%) ammonia hydrate  $NH_4OH$ . The resulting solution is of an intensely blue color and may be considered to be merely a mixture of cupric-oxide, ( $CuO$ ) ammonia ( $NH_3$ ) and water.

We have found even under adverse conditions that with about two amperes per square inch of anode, that we can obtain about forty grams of cellulose and about twenty-three and one-half grams of copper in about an hour and a half. This however is not

submitted as an accurate statement as to what may be done under more favorable conditions.

Of course it will be understood that changes may be made in the various ingredients and proportions thereof and in the manner of manipulating the same without departing from the spirit of the invention as claimed.

We claim:

1. A method of dissolving organic material while in a cellular or fibrous condition or which has been in such condition, in a solvent containing a plurality of combined chemical elements, at least one of said elements being a metal, and at least one being volatile, passing the resultant colloidal solution through an electrolytic field or fields thereby causing the metallic constituent to be electrolytically extracted and deposited upon one electrode, the volatile constituent to be released from solution, and the organic material to be deposited on the other electrode in a homogeneous condition without change in its original chemical constitution.

2. A method of dissolving organic material while in a cellular or fibrous condition or which has been in such condition, in a solvent containing a plurality of combined chemical elements, at least one of said elements being a metal, and at least one being volatile, passing the resultant colloidal solution through an electrolytic field or fields thereby causing the metallic constituent to be electrolytically extracted and deposited upon one electrode, the volatile constituent to be released from solution, and the organic material to be deposited on the other electrode in a homogeneous condition without change in its original chemical constitution, and providing means for recovering both metallic and volatile constituents and returning them together with successive portions or quantities of organic material to the electric field.

3. A method of dissolving organic material and placing same in solution on a moving carrier, causing said material to deposit as a homogeneous solid on the carrier by means of an electric current, removing the solid material from the carrier and improving its physical character by means of volatile solvents combined with mechanical pressure.

4. A method of dissolving cellular or fibrous organic material in a solvent containing a plurality of chemical elements, at least one of said elements being a gas, placing the solution on a continuously moving carrier surrounded by a moving atmosphere of the said gas in a dry condition thereby tending to concentrate the solution of organic material and preventing access of external deleterious gases or substances, allowing the organic material to remain in this

- atmosphere until it is in a homogeneous state returning the gas to its source of supply and removing the homogenous material.
5. The method of producing cellulose which consists in dissolving organic matter in a suitable solvent, flowing the solvent carrying the dissolved organic matter into a sheet or film and then subjecting the sheet or film to electrical action.
10. 6. In an apparatus of the class described, an endless conveyer, a chamber through which said conveyer serving as an electrode travels through which material may be fed upon said conveyer to form a film, means for passing said film through an electrolyte provided with electrodes, means for extracting the metallic content of said film through said electrolyte, means for thereafter washing said film, means for thereafter drying said film, means for thereafter finally separating and treating said film.
15. 7. In an apparatus of the class described, an endless conveyer, a chamber through which said conveyer serving as an electrode travels through which material may be fed upon said conveyer to form a film, means for passing said film through an electrolyte provided with electrodes, means for extracting the metallic content of said film through said electrolyte, means for thereafter washing said film, means for thereafter drying said film, means for thereafter finally separating and treating said film, and in combination, means for recovering the materials used in the treatment of said film.
20. 8. The method of treating cellulose material which consists in providing an anode carrier, in an electrolytic cell with a solution of the cellulose material between the cathode of the cell and said anode carrier, and passing a direct current through the cell from one of said electrodes to the other, and finally stripping the cellulose from the anode carrier.
25. 9. The method of treating cellulose material which consists in passing an anode carrier through an electrolyte in an electrolytic cell, and electrolyzing the cellulose on said carrier as it passes through the electrolyte.
30. 10. The method of treating organic material which consists in passing a carrier for the material continuously through the electrolyte of an electrolytic cell, and electrolyzing the organic material on the carrier as it passes through the electrolyte.
35. 11. The method of treating cellulosic material which consists in passing a carrier for the material continuously through the electrolyte of an electrolytic cell, electrolyzing the cellulose on the carrier as it passes through the cell, and without stopping passing the electrolyzed cellulose through a washing bath.
40. 12. The method of treating organic material which consists in passing a carrier for the material continuously through the electrolyte of an electrolytic cell, electrolyzing the cellulose on the carrier as it passes through the electrolyte, the material continuously through the electrolyte of an electrolytic cell, electrolyzing the organic material on the carrier as it passes through the electrolyte, and without stopping passing the material through means subjecting the material to further treatment.
45. 13. The method of treating cellulose material which consists in passing an anode carrier through an electrolyte in an electrolytic cell, electrolyzing the cellulose on said carrier as it passes through the electrolyte, and without stopping passing the treated cellulose through a washing bath and drying apparatus consecutively.
50. 14. The method of treating cellulosic material which consists in placing a layer of the cellulosic material on a carrier, and moving the carrier through the electrolyte of an electrolytic cell, electrolyzing the cellulose on said carrier as it passes through the electrolyte.
55. 15. The method of treating cellulose material which consists in passing an anode carrier through an electrolyte in an electrolytic cell, electrolyzing the cellulose on said carrier as it passes through the electrolyte while maintaining the cell closed to the outside atmosphere.
60. 16. The method of treating cellulose material which consists in passing an anode carrier through an electrolyte in an electrolytic cell, electrolyzing the cellulose on said carrier as it passes through the electrolyte, and without stopping passing the treated cellulose through a washing bath and drying apparatus consecutively, the cellulose being kept substantially free of  $\text{CO}_2$  while passing through the electrolytic cell, washing bath and drying apparatus.
65. 17. The method of treating cellulosic material which consists in placing a layer of the cellulosic material on a carrier, and moving the carrier through the electrolyte of an electrolytic cell, electrolyzing the cellulose on said carrier as it passes through the electrolyte, and keeping the cellulosic material substantially free of  $\text{CO}_2$  of the air after it is placed on said carrier and until it has left said cell.
70. 18. The method of treating cellulose which consists in preparing a solution of cellulosic material, placing same on a moving carrier in an atmosphere of an inert gas, and passing the carrier through an electrolyte, electrolyzing the cellulose on the carrier.
75. 19. The method of treating cellulose which consists in preparing a solution of cellulosic material, placing same on a moving carrier in an atmosphere of an inert gas, and passing the carrier through an electrolyte, electrolyzing the cellulose on the carrier, said electrolyte being in a cell closed to the outside atmosphere.
80. 20. The method which consists in passing an electrode carrier through an electrolytic

cell and treating a solution of cellulosic material electrolytically in said cell whereby solvent constituents are removed from said solution electrolytically and cellulose is carried from the cell on the carrier.

21. The method of treating cellulosic material which consists in preparing a thick solution thereof, applying a layer of the solution to an endless band, and passing said band through an electrolytic cell in which it forms the anode, thereby electrolyzing the cellulose on said band.

22. The method of treating organic material which consists in applying a thick solution of the organic material to a moving carrier, and passing the solution on the carrier through an electrolyte in an electrolytic cell, thereby electrolyzing the solution on the carrier.

23. The method of treating cellulosic material which consists in dissolving the same, concentrating the solution thereof, applying the concentrated solution to a moving carrier and passing the solution on the carrier through an electrolyte in an electrolytic cell, thereby electrolyzing the solution on the carrier.

24. The method of treating cellulosic material which consists in preparing a solution of the cellulosic material with a metallic salt solvent, applying the solution to a moving carrier, passing the solution on the carrier through an electrolytic bath, thereby

electrolyzing the solution on the carrier and depositing the metal of the salt on a cathode 35 in the electrolytic bath, the carrier forming an anode on which the cellulose is electrolyzed.

25. The method of treating cellulosic material which consists in preparing a solution 40 of the cellulosic material, passing a carrier through an electrolytic cell and electrolyzing the cellulose on the carrier as it passes through the electrolytic cell.

26. The method of treating cellulosic material which consists in subjecting the same to electrolysis to deposit the cellulose electrolytically and treating cellulose with a volatile organic softening agent.

27. The method of treating cellulosic material which consists in subjecting the same to electrolysis to deposit the cellulose electrolytically and treating cellulose with amylo-acetate.

28. The method of treating cellulosic material which consists in preparing a solution 55 of the cellulosic material, applying said solution to a moving carrier, moving the solution on said carrier through an atmosphere of ammonia into an electrolytic bath and electrolyzing the cellulose on the carrier therein.

In testimony whereof we hereunto affix our signatures.

EDWIN TAYLOR.

EDWARD F. CHANDLER.